

## UNITED STATES PATENT OFFICE

1,935,321

## GUTTA-PERCHA INSULATION MATERIAL

Archie R. Kemp, Westwood, and John H. Ingmanson, Bloomfield, N. J., assignors to Bell Telephone Laboratories, Incorporated, New York, N. Y., a corporation of New York

No Drawing. Application February 3, 1930  
Serial No. 425,710

8 Claims. (Cl. 18—49)

This invention relates to gutta-percha insulation materials and to methods of producing such materials, and more particularly to improvements in materials of this kind for use in long deep sea cables especially designed for higher frequencies than the usual cable telegraph signaling frequencies.

It is an object of the invention to provide an insulating material comprising gutta-percha which has better electrical properties than gutta-percha insulation hitherto employed in deep sea cables and which is suitable for use in long cables designed for telephone frequencies or even for higher carrier current frequencies.

Another object of the invention is to provide an improved gutta-percha as a compounding material for deep sea cable insulation material which has electrical properties as good as or better than practically pure gutta-hydrocarbon.

Another object of the invention is to provide an improved gutta-percha of this kind which besides having satisfactory electrical properties has improved mechanical properties.

Still another object is to provide a method of treating gutta-percha whereby inferior grades may be brought up to standard requirements as to mechanical properties as well as to electrical characteristics; or whereby such inferior gutta-percha may be improved to have, besides the required mechanical properties, better electrical characteristics than those usually required for even high speed telegraph submarine cables.

Still another object is to provide a method of producing such a material which is commercially feasible.

For the purpose of the present specification, and the claims appended thereto, the term gutta-percha includes the various grades of balata.

In accordance with the invention gutta-percha is treated in such a manner that it is deprived of certain of its resinous constituents which have been found to have unsatisfactory electrical properties under certain sea bottom conditions, and other resins, naturally present in the gutta-percha or else obtained from other sources and which have been found to have satisfactory electrical properties, are utilized in the gutta-percha product to add thermo-plastic characteristics thereto, and possibly to afford a protective action, as well as to improve its electrical characteristics.

The mechanical properties which in present day practice are required of the compound comprising the main insulating body in deep sea cables include thermo-plasticity, ability to be extruded in a uniform fashion around the conductor at the usual extrusion temperatures, limited cold flow at room and sea bottom temperatures, toughness and flexibility at room temperatures, etc. The mechanical properties of the component substances of the insulating compound may, of course, differ somewhat from these standards, inasmuch as these substances usually are chosen with regard to their ability to complement each other in this respect.

An important electrical characteristic of the insulating material is the leakance factor G/C, which is the ratio of leakance to capacity of a sample. This factor is of greater importance as the frequency of the applied current increases and it should be kept low under sea bottom conditions to insure a low attenuation of signals over a long cable.

It has before been known that gutta-percha, and therefore also balata, can be improved electrically by the removal of resins therefrom. It has therefore been concluded that the resins themselves have less satisfactory electrical properties than has the gutta-hydrocarbon.

The resins of gutta-percha, including those of balata, have before been separated and certain of their physical and chemical characteristics have been determined. They have been found to fall into two main groups, termed fluavil and albane, sometimes spelled alban. The albane fraction is usually a white crystalline material and may be further separated into a series of fractions having different melting points. It is soluble in hot alcohol and in petroleum naphtha, but is nearly insoluble in cold alcohol. The fluavil fraction is a yellow product melting at low temperatures and soluble in cold alcohol as well as in petroleum naphtha.

In an investigation conducted in an attempt to determine how gutta-percha, and particularly balata, may be improved for the purpose of deep sea cable insulation, we have found that the less satisfactory electrical properties may be ascribed particularly to the resins included in the fluavil group or to some constituent contained in or intimately associated with the fluavil, whereas



|                  | Per cent<br>by weight |
|------------------|-----------------------|
| Moisture content | 1.34                  |
| Resinous content | 4.1                   |

5 Electrical tests at 0° C. gave the following data:

|    | f         | G/C | K    |
|----|-----------|-----|------|
| 10 | 1000 c/s  | 39  | 2.75 |
|    | 3000 c/s  | 112 | 2.74 |
|    | 10000 c/s | 360 | 2.72 |

Sample G.—A whole resin extracted from balata was subjected to electrical tests at 0° C. 15 and gave the following data:

|    | f         | G/C   | K    |
|----|-----------|-------|------|
| 20 | 1000 c/s  | 53.9  | 3.26 |
|    | 2000 c/s  | 180.5 | 3.25 |
|    | 3000 c/s  | 367   | 3.24 |
|    | 10000 c/s | 2540  | 3.17 |

Sample H.—75 grams of a whole balata resin 25 was subjected to an extraction for 6 hours at room temperature in 900 cm<sup>3</sup> of ethanol after which it was filtered and the residue washed in ethanol and the alcohol carefully removed.

Electrical tests at 0° C. gave the following data:

|    | f         | G/C  | K   |
|----|-----------|------|-----|
| 30 | 1000 c/s  | 11.6 | 2.2 |
|    | 2000 c/s  | 21.3 | 2.2 |
|    | 3000 c/s  | 50   | 2.2 |
| 35 | 10000 c/s | 69.3 | 2.2 |

The Sample H, which constituted the undissolved residue from the cold alcohol extraction 40 of balata resins, was a white crystalline material having the characteristics of the albanes with a melting point range of 165° C. to 195° C.

By adding the albane Sample H to the substantially resin free gutta-hydrocarbon Sample 45 F in proportions determined by the requirements, an insulating material may be obtained which combines electrical properties better than those of the original product represented by Sample A and in some respects better than those 50 of the deresinated balata of Sample F with mechanical properties satisfactory for deep sea cable insulation.

Though the various samples described had all 55 been taken from balata, similar treatments may be given to any other type of gutta-percha with corresponding results. It is furthermore possible to extract and separate the albanes from any one or more gutta-percha varieties and use them in the desired proportions as plasticizing 60 agents for any one variety or combination of varieties of gutta-percha. Again, other natural albanes or albane rich substances may be incorporated by well known mixing processes as a plasticizing agent in any of these instances, such 65 as chicle or the albanes of chicle.

It is obvious that the temperatures at which the fluavil extraction from gutta-percha is made may be somewhat different from room temperatures depending upon the solvent used, the time 70 allowed for the extraction and upon the degree of extraction desired. Thus a very quick extraction may be made with methanol at temperatures as high as 60-65° C. Besides the preferred solvents, methanol and ethanol, a number of other solvents may be used such as propyl alcohol, acetone,

methyl ethyl ketone, as well as mixtures of some of these. By the proper choice of the three factors mentioned above, it is possible to extract more or less of the fluavil constituent and also certain of the albanes from the albane constituent of the gutta-percha.

Various methods described as examples of this invention have involved the removal of fluavil from the gutta-percha. It is possible that the poor electrical properties of fluavil are not inherent to the main bulk of the fluavil but are due to smaller quantities of substances which are more closely associated with the fluavil than with the albane and which may be less easily separated therefrom. Thus the fluavil extractions have been found to contain small quantities of free acids and still smaller quantities of free alcohol. These quantities appear, however, to be sufficient to justify the assumption that one or both of these substances are the cause of the degradation in the electrical properties of gutta-percha.

It should be understood that the mechanical properties of any particular body of gutta-percha which is suitable for incorporation in a 100 cable insulating material are not necessarily identical with the mechanical properties required for such insulating material. By the methods forming part of this invention any quality of gutta-percha, which in present practice is considered suitable for use in admixture with other qualities of gutta-percha or with other compounding materials may have its electrical properties improved and at the same time may retain its mechanical properties or even have these 105 somewhat improved.

It is within the scope of this invention to admix with the above described gutta-hydrocarbon and albane composition such materials as: natural rubber of all sorts treated or untreated to 115 remove objectionable constituents, such as soluble salts and proteins; synthetic rubber prepared by polymerizing any of the known conjugated dienes; waxes which are derived from natural sources or prepared synthetically; anti-120 oxidants such as phenyl alpha napthylamine or phenylbeta-napthylamine or any other product which may act to modify the properties of the gutta-hydrocarbon and albane composition in the direction to attain the desired product.

What is claimed is:

1. A gutta-percha product comprising resin poor gutta-percha in which albane has been incorporated as a plasticizing agent.
2. A gutta-percha product comprising a great-130 ly deresinated gutta-percha and as a plasticizing agent a foreign albane, such as chicle albane.
3. A gutta-percha product in which resins having better electrical properties have replaced natural resin constituents having poorer electrical 135 properties.
4. A method of improving the electrical properties of gutta-percha which comprises extracting at least a portion of the resins therefrom, separating from the extracted resins at least a portion of those constituents which have the poorer electrical properties and restoring a portion of the remaining constituents to the gutta-percha.
5. A method of treating gutta-percha which comprises extracting a portion of the resins there-145 from, separating the albanes from the extract and incorporating said separated albanes in the gutta-percha from which resin was removed.
6. A method of improving the mechanical properties of at least partially deresinated gutta-150

percha by mixing a quantity of albanes therewith.

7. A method of improving the electrical properties of gutta-percha which has been considerably deresinated which comprises mixing a foreign substance therewith, the main natural constituent of which is albane.

10

15

20

25

30

35

40

45

50

55

60

65

70

75

8. A method of improving the electrical and mechanical properties of gutta-hydrocarbon by mixing therewith an albane rich substance such as chicle.

ARCHIE R. KEMP.  
JOHN H. INGMANSON.

80

85

90

95

100

105

110

115

120

125

130

135

140

145

150